

# UNITED STATES PATENT OFFICE.

THURSTON C. MERRIMAN, OF NEW HAVEN, CONNECTICUT, ASSIGNOR TO WINCHESTER REPEATING ARMS CO., OF NEW HAVEN, CONNECTICUT, A CORPORATION.

## SURFACE-COLORED ARTICLE OF COPPER ALLOY.

1,327,400.

Specification of Letters Patent.

Patented Jan. 6, 1920.

No Drawing.

Application filed August 5, 1919. Serial No. 315,448.

*To all whom it may concern:*

Be it known that I, THURSTON C. MERRIMAN, a citizen of the United States, residing at New Haven, in the county of New Haven and State of Connecticut, have invented a new and useful Improvement in Surface-Colored Articles of Copper Alloy; and I do hereby declare the following to be a full, clear, and exact description of the same.

10 My invention relates to an improved surface-colored copper alloy, the object being to produce for any available purpose, at a low cost for production, articles of copper alloy having a durable and handsome black, 15 or substantially black, surface color.

With these ends in view my invention consists in a copper alloy containing arsenic, provided with a surface finish of black, or substantially black, color, and in certain 20 details and characteristics, as will be herein-after described and pointed out in the claims.

In carrying out my invention, I employ a copper alloy containing a small amount of arsenic. I have secured satisfactory results with an alloy consisting of 70 parts of copper, 29 parts of zinc, and 1 part of arsenic; but I do not limit myself to such ingredients or proportions; though my present belief is that the percentages of copper and 25 arsenic should be held around those above stated. The other ingredients will be varied according to circumstances, *i. e.*, as to the cost, form, character and use of the article.

An article of such characterization—that 30 is, characterized as an alloy of copper containing arsenic, having been thoroughly cleaned, is first immersed in an acid oxidizing bath which may be composed as follows:

40 100 cc. water.

25 cc. nitric acid (1.42 sp. gr.)

5 gms. potassium dichromate.

In this first bath, the article is allowed to remain about five minutes at "room temperature" after which it is removed and thoroughly rinsed in clear cold water. The article is then subjected to an acid solution containing a sulfid and an arsenious compound. The second bath may be composed 45 as follows:

710 cc. water.

237 cc. hydrochloric acid (1.2 sp. gr.)

1.1 grams potassium sulfid.

170 grams arsenious oxid.

55 In this second bath, the article is allowed

to remain about five minutes at a temperature of between 140-155 degrees F., after which the article is removed, thoroughly rinsed in cold water, dried and given a thin coat of light oil. The article as thus treated, 60 will be provided with a durable and handsome surface finish of black, or substantially black, color.

I do not limit myself, as already stated, to any particular alloys, so long as they 65 contain copper and arsenic, nor do I limit myself to compounding the two solutions in accordance with the formulæ given, as the ingredients and their proportions may be varied as may be required by their character 70 and strength, as well as by the specific character of the alloy used, nor do I limit myself to the times and temperatures stated, as those factors will vary with the other variations suggested as falling within the 75 purview of my invention, my present invention being characterized by producing upon the surface of an alloy containing copper and arsenic, a remarkably permanent and handsome surface finish of black, 80 or substantially black, color by the use of an acid oxidizing bath followed by a bath containing a sulfid and an arsenious salt. In my co-pending application filed August 5, 1919, Serial #315449, I have claimed the 85 process by means of which I produce the articles hereinafter described.

I claim:

1. As a new article of manufacture, an article of copper alloy containing arsenic and 90 having a surface finish of black, or substantially black, color.

2. As a new article of manufacture, an article composed of an alloy containing substantially 70% copper, 29% of other metals, 95 and 1% arsenic, and having a surface finish of black, or substantially black, color.

3. As a new article of manufacture, an article composed of an alloy containing substantially 70% copper, 1% arsenic, and 100 29% of zinc, and having a surface finish of black, or substantially black, color.

In testimony whereof, I have signed this specification in the presence of two subscribing witnesses.

THURSTON C. MERRIMAN.

Witnesses:

ARTHUR W. EARLE,  
ERIK S. PALMER.